

## UNITED STATES PATENT OFFICE

2,632,562

CONTAINER AND TREATING APPARATUS  
FOR SOUR CRUDE OILS

Clarence H. Dragert, Dallas, Tex.

No Drawing. Application June 9, 1948,  
Serial No. 32,050

3 Claims. (Cl. 206—2)

1

This invention relates to improved methods for storing and treating sour crude oils and for providing improved tanks and apparatus for this purpose.

Such sour crude oils contain varying amounts of sulphur compounds and varying amounts of emulsified water, and, under the usual conditions of storage in steel tanks, rapidly attack the metal of such containers by corrosion. Even the upper portions of such containers, which are not in direct contact with the liquid oil, are attacked by the fumes of the contents, so that they are rendered unfit in a relatively short time and require frequent replacement, thus adding greatly to the annoyance and cost of properly storing and treating the oils of this grade. It is not unusual, under intensive use, that heavy metal tanks and piping require replacement within as short a time as thirty days, and they seldom remain fit for service beyond a few months.

The conditions are especially severe where oil treatment is necessary. If the oil comes from the ground as an emulsion with water, such oil must often be treated to break the emulsion. This is done with what is known as an "oil treater." Such "treaters" are tall tanks which contain a heating unit which heats the contents to about 140° F.

While the mere storing of the sulphur containing sour crude oils is destructive of the containers in a relatively short time, the corrosion proceeds at an even more rapid rate in this treating process.

It has long been a problem for the operator, in this particular field to find satisfactory means for coating the inner surfaces of the drums used for storage and the tanks employed for "treating" these sour crude oils. Many different oils, paints, cements, and other compositions and devices have been tried as protective means but with little avail.

Thus, steel shells have been made heavier with the possible expectation that, after the corrosion proceeded to a degree, the corrosion crust would itself act as a retardant against further destructive action before the metal was too deeply affected; heavy paint coverings and inner cement shells have been applied; and various forms of rubber coatings have also been tried. But none of these various methods have produced any really effective economies. The heavier steel took somewhat longer for perforation, but the higher costs cancelled any gain in the longer time for re-installation. Ordinary paints, containing lead oxide, carbonate or sulfate, are soon eaten away and even the inner cement shells crack and fall off, while the rubber coatings blister and peel off very soon. Metallic coating, as by galvanizing,

2

has also failed in producing any satisfactory solution of this problem.

It has now been discovered by the applicant that the life of the steel storage drums and treating tanks and the like, can be considerably prolonged for practical periods and to such a degree as to result in substantial economies for this industry both in the materials and in the expense for re-installations. This improvement is attained by the application of an adhesive coating carrying metallic lead powder in sufficient concentration so as to afford substantially uniform deposits of the lead metal.

With such a protective lead-powder coating, containers have been in very prolonged operation and some such are still in active use without discoverable depreciation.

The compositions of the coating agents which are useful for adaptation to the practice of my invention herein, comprise finely divided lead metal, dispersed in various liquid media such as are generally employed for protective coatings by themselves or which serve as vehicles for carrying ordinary paint pigments, such as lead carbonate, oxide, and sulfate. Various useful types of vehicles as are illustrated herein may be modified considerably both as to components and as to their relative proportions, as a matter of choice for adaptation to special conditions. The important and controlling constituent in all such compositions is the finely divided lead metal, which has been found to be the practical protective agent against this destructive sour crude oil liquid and its fumes.

The choice as to carrier composition may be determined to a large degree by local conditions, and the special compositions of the particular types of the sour crude oil being treated. In general, the guiding principle is to provide means for good binding, distribution, dispersion and suspension, and the carrying and suspending medium should also be substantially inert to the action of the sulphur compounds contained in the oil.

A serviceable coating composition which has proved effective is prepared with

100 pounds of esterified rosin  
25 gallons of China-wood oil  
300 pounds of thinner

After "cooking" in the conventional manner, about 14 pounds of finely divided lead powder are added per gallon of liquid with active stirring until the metal is well dispersed throughout. The mixture is then ready for application to the surfaces to be treated.

The China-wood oil has been serviceably sub-

stituted by other oils, such as oiticica, linseed, dehydrated castor oil, perilla and soya bean oil, also fish oil.

Similarly, substitution has been made for the esterified rosin, in the form of cumar resin derived from coal tar, pure and modified phenolic resins, maleic acid type resins, etc.

Another type of composition which has been employed successfully, embraces the use of alkyd resins, such as are derived by the action of polybasic acid on polyhydric alcohols. Still another type of vehicle is that which has been obtained by using the polymerized products from vinyl acetate, vinyl chloride, polystyrene, chlorinated rubber, etc. Such polymers, when plasticized and formulated with some hard resin to effect adhesion, serve well as covering agents.

When used along, or with the usual lead paint pigments, such coatings do not protect the interiors of vessels containing the sour crude oils, from the ravages of corrosion. However, when any of these several types of coating media are used as carriers for the lead powder as disclosed herein, there is provided a coating which serves definitely for protection against such corrosion.

The viscosity may also be suitably controlled for adaptation to brushing or spraying within practical limits, but with due regard to the proper and even dispersion and suspension of the lead powder.

The amount of lead powder in such mixtures is preferably from about 12 to 14 pounds of lead to the gallon of liquid. For convenience in handling and application this amount may optionally also be varied within practical limits. Obviously, when less of metal powder is included in a given batch, this may require the application of more coats for effective coverage and hiding of the surfaces to be protected.

The metallic lead ingredient may also be employed in varying degrees of fineness from as much as about 200 mesh to a practically impalpable powder, depending upon the service expected, the character of the surfaces to be covered, the number of coats deemed desirable, and the method of application as by brushing for instance or by spraying. Obviously, the finer the lead powder the better the suspension and dispersion. Depending on these variable factors, also a greater or less number of coats may be superimposed so as to attain satisfactory and practical over-all coverage of the surfaces to be coated, with the lead.

It is highly desirable that the lead metal powder, as used in preparing the mixture, should be freshly prepared or should be protected against air and moisture so as to avoid any substantial chemical change in the metal, as by oxi-

dation. Any considerable amount of oxidation is detrimental.

It is a noteworthy fact, that these same lead-metal coatings herein disclosed have not been found effective as protective agents against corrosion of metallic exteriors of plant equipment and apparatus in chemical laboratories, which are exposed to the fumes of sulphuric acid and hydrogen sulfide. Yet, when these same compositions which have thus been found ineffective on such exteriors are coated upon the interiors of the sour crude containers, definite protection is afforded by such coatings for prolonged periods.

15 I claim:

1. The process of storing and treating sour crude oils which comprises introducing such oils into a container whose body is composed of ferrous material which reacts destructively with the acidic and sulfurous constituents of these oils, but which has the inner surfaces substantially evenly covered with a coating comprising finely comminuted lead metal.

2. The process of storing and treating sour crude oils which comprises introducing such oils into a container whose body is composed of ferrous material which reacts destructively with the acidic and sulfurous constituents of these oils, but which has the inner surfaces substantially evenly covered with a coating comprising finely comminuted lead metal, substantially free from oxide.

3. The process of storing and treating sour crude oils which comprises introducing such oils into a container whose body is composed of ferrous material which reacts destructively with the acidic and sulfurous constituents of these oils, but which has the inner surfaces substantially evenly covered with a coating comprising finely comminuted lead metal, substantially free from oxide, and binding material substantially inert to such crude oil acids and sulfur compounds.

CLARENCE H. DRAGERT.

#### REFERENCES CITED

The following references are of record in the file of this patent:

#### UNITED STATES PATENTS

| Number    | Name                     | Date          |
|-----------|--------------------------|---------------|
| 1,210,375 | Decker                   | Dec. 26, 1916 |
| 1,717,140 | Brandenberger            | June 11, 1929 |
| 1,911,696 | Lerio, Jr.               | May 30, 1933  |
| 1,961,936 | Mallinkrodt, Jr., et al. | June 5, 1934  |
| 2,041,392 | Bean                     | May 19, 1936  |
| 2,245,745 | Ball                     | June 17, 1941 |
| 2,346,714 | Wobbe                    | Apr. 18, 1944 |